

# UNITED STATES PATENT OFFICE.

ANASTAZA KOSZYCZAREK, OF CLEVELAND, OHIO.

## LUBRICATING COMPOSITION FOR INTERNAL-COMBUSTION ENGINES.

No Drawing.

Application filed January 14, 1924. Serial No. 686,203.

To all whom it may concern:

Be it known that I, ANASTAZA KOSZYCZAREK, a citizen of the United States, residing at Cleveland, in the county of Cuyahoga and State of Ohio, have invented certain new and useful Improvements in a Lubricating Composition for Internal-Combustion Engines, of which the following is a specification.

10 This invention relates to an improvement in a lubricating composition for internal combustion engines, the general object being to provide a lubricating mixture, which will under the varying conditions arising in an 15 internal combustion engine operating an automobile have the power to maintain an unbroken film for long periods of use, and not leave, in evaporating, any residue or cause objectionable carbonization of the oil 20 due to the high temperature of the walls and presence of flame in the engine.

The composition consists of a preponderating amount of pure mineral lubricating oil derived from crude petroleum by fractional 25 distillation, a small amount of oil or spirits of turpentine, and a lesser amount of a vegetable, non-drying oil. The mineral lubricating oil may be any one of the series of lubricating oils derived from crude petroleum 30 by distillation or other refining processes, preferably a medium mineral lubricating oil having a flash point of 325° to 350° F., a fire point of 370° to 390° F., and a viscosity of 275 to 310 seconds at 100° F. (Sayboldt.)

The vegetable non-drying oil is preferably 35 olive oil of a pure grade adapted to be heated to a high temperature without undergoing chemical change or conversion into hydrocarbons when mixed with mineral lubricating oil, and a terpene product. A 40 miscible composition made according to my invention, may consist of fifty to sixty parts of lubricating oil, two to four parts of turpentine, and one to two parts of olive oil. A 45 preferred mixture consists of seven gallons of medium lubricating oil, one quart of refined spirits of turpentine, and one pint of pure olive oil. This specific composition gives highly satisfactory results as a non- 50 carbonizing lubricant for automobile engines, that is to say, it has been demonstrated that this mixture provides an excellent lubricant for an internal combustion engine without forming carbon deposits in 55 the cylinders.

What I desire to claim, is:

A lubricating composition for internal combustion engines comprising approximately fifty to sixty parts of a medium lubricating oil, approximately two to four 60 parts of oil of turpentine, and approximately one to two parts of olive oil.

In testimony whereof I affix my signature in presence of two witnesses.

ANASTAZA KOSZYCZAREK.

Witnesses:

VIRGINIA MOSER,  
Mrs. HATTIE WESOLOWSKI.